

## UNITED STATES PATENT OFFICE

2,495,225

METHOD FOR THE PRODUCTION OF LOW  
SULFUR SPONGE IRONRussell C. Buehl, Edgewood, and John P. Riott  
and Earle P. Shoub, Pittsburgh, Pa.No Drawing. Application October 7, 1947,  
Serial No. 778,452

1 Claim. (Cl. 75—33)

(Granted under the act of March 3, 1883, as  
amended April 30, 1928; 370 O. G. 757)

1

The invention described herein may be manufactured and used by or for the Government of the United States for governmental purposes without the payment to us of any royalty thereon in accordance with the provisions of the act of April 30, 1928 (Ch. 460, 45 Stat. L. 467).

This invention relates to the production of easily reducible metals from their ores, and more particularly to the production of such metals having a low sulfur content. Still more particularly this invention relates to the production of metallic iron and similar metals of the iron group of the periodic system wherein the final product has a low sulfur content.

In processes for the production of various easily reducible metals of a low sulfur content, particularly rotary kiln sponge iron processes, various alkaline earth compounds have been employed and suggested as applicable for use as desulfurizing agents. Such processes have been described and extensively referred to in the Bureau of Mines Bulletin 270 (1927), U. S. Patent 2,380,406 (Buehl), and other well known literature.

The Buehl patent discloses the use of a pre-calcined mixture of coal and either lime, dolomite, or other alkaline earth compounds ground to pass a 10-mesh screen for the production of low sulfur sponge iron. This method involves the calcining of the coal and the sulfur control agent and this operation adds to the cost of the process.

Accordingly, it is an object of this invention to provide a method for the production of low sulfur content metals from their ores, which is inexpensive and does not involve any special processes which add appreciably to the cost.

It is another object of the invention to provide a metallurgical composition for the production of low sulfur metallic iron. It is still another object of the invention to provide desulfurizing agents for use in the production of low sulfur metals. Other objects and advantages will be apparent or will appear hereinafter.

These objects and advantages are accomplished in accordance with this invention through the use of dolomite sized to about minus 8 plus 100 mesh as desulfurizing agent.

Suitable processes wherein sized dolomite may be employed as a desulfurizing agent in accordance with this invention include the processes for the reduction of ores of metals with coke or other carbonaceous reducing agents at elevated temperatures. Examples of such process are those for the production of metallic iron, copper, cobalt, nickel, cadmium, and other metals which

2

can be reduced from their oxides, carbonates, and the like, with carbonaceous reducing agents such as charcoal, coals, petroleum, coke, bitumen, bituminous coals having coking characteristics, and the like. In general processes for the treatment of ores of the metals of the iron group in periodic system can best be treated in accordance with this invention, and of these, processes for the production of sponge iron in a rotary kiln constitute preferred members.

In a typical embodiment of the preferred rotary kiln process for the production of the sponge iron a mixture of the raw materials in granular form is fed into the elevated end of the kiln, which is fired axially from the lower or discharge end. In the reducing zone, which is approximately one third the length of the kiln measured from the discharge end, a temperature of 1800° to 2000° F. is maintained. The reduced material is discharged through a cooling chamber, which is an integral part of the kiln and which prevents the material from being reoxidized by air during cooling. This discharge is then passed through a magnetic separator, which removes the magnetic sponge iron from the non-magnetic char and desulfurizing agent.

A study was made of the form in which sulfur exists in sponge iron and of the factors that influence the transfer of sulfur into the sponge iron when solid reducing agents are employed. It was indicated that if no sulfur-controlling agents were employed, sulfur contents as high as 0.25 per cent could be expected. The addition of lime, limestone, or dolomite in powdered form to the feed did not lower the sulfur content sufficiently to make the sponge iron desirable as a melting stock. In contrast to these results, the addition of sized dolomite to the feed reduced the sulfur content to the range of 0.02 to 0.05 per cent. Sized lime, while beneficial, was not nearly as effective as sized dolomite, sulfur contents being in the range of 0.04 to 0.07 per cent. This difference in the results is attributed to the tendency of the particles of lime to be pulverized by tumbling and the abrasive action of the charge in the kiln. Limestone is converted to lime at the operating temperature and therefore loses its physical strength. In contrast, dolomite retains its physical strength when heated, therefore, the particles do not crumble in the rotating kiln. As a result of the pulverizing action in the rotary kiln, fine particles of basic desulfurizing agent adhere to the surface of the sponge-iron granules, and this surface coating has been found to contain most of the sulfur in the sponge-iron product.

An accurate sulfur balance is difficult to obtain because of sulfur loss in the combustion gases. An approximate sulfur distribution is given below for a charge consisting of equal parts of low sulfur magnetite ore (0.02 per cent S) and coke (0.8 per cent S) with the addition of sized dolomite to the extent of 10 per cent of the weight of the ore. Sponge iron with a sulfur content of 0.03 per cent was produced in an internally fired rotary kiln from these raw materials. In this event, low-sulfur oil (0.3 per cent S) was used to supply the heat for the process. With these raw materials, over 90 per cent of the sulfur in the charge is contained in the reducing agent. About 2.5 per cent of the sulfur in the charge appears in the sponge iron, 60 to 70 per cent of the initial sulfur remains in the unconsumed coal and coal ash rejected by the magnetic separator, 16 per cent is contained in the dolomite, and the remainder passes off to the combustion gases. When no desulfurizing agent is employed, the sponge iron contains from 16 to 20 per cent of the sulfur in the charge.

A partial summary of experimental evidence to demonstrate the existence of a basic coating containing most of the sulfur in the sponge-iron concentrate is presented in the following paragraphs, and will show how the invention may be carried out, but is not limited thereto.

*Example*

Sponge iron was produced in an externally heated, horizontally rotating alloy retort 8 inches in diameter and 15 inches long. Samples were prepared using minus 8-mesh unsized dolomite, minus 8 plus 100-mesh dolomite and a control wherein no desulfurizing agent was used.

*Control.*—(a) Sponge iron was prepared from a mixture of 2 kg. of Chateaugay ore and 1.5 kg. of No. 4 anthracite (0.7 per cent sulfur) with no desulfurizing agent employed. The sponge iron so produced contained 0.07 per cent sulfur before sizing and the sulfur appears to be uniformly distributed through the sponge iron particles.

*Unsized dolomite.*—(b) Sponge iron was produced from the same mixture of iron ore and coal, except that 0.3 kg. of minus 8-mesh unsized dolomite was added as the desulfurizing agent. The dolomite had the normal size distribution that results from grinding, and contained 42 per cent of minus 100-mesh material. The sulfur content of this sponge iron was 0.077 per cent, and is about the same as when no dolomite is employed.

*Sized dolomite.*—(c) Sponge iron was made from a similar charge of ore and anthracite, but with the addition of minus 20 plus 100-mesh dolomite to the extent of one fifteenth the weight of the coal. The addition of the sized dolomite reduced the sulfur content of the sponge iron to 0.019 per cent.

The results after sizing of the sponge iron products so produced are tabulated below in part as the table.

Table.—Percent sulfur in sponge iron fractions

|                            | Sponge iron particle size range (mesh) |        |         |          |
|----------------------------|----------------------------------------|--------|---------|----------|
|                            | -20+48                                 | -48+65 | -65+100 | -100+200 |
| No dolomite.....           | 0.07                                   | 0.07   | 0.07    | 0.06     |
| -8 mesh dolomite.....      | 0.06                                   | 0.10   | 0.16    | 0.57     |
| -20+100 mesh dolomite..... | 0.016                                  | 0.017  | 0.023   | 0.06     |

If a surface layer containing a high sulfur content is present on the particles, finer sized particles will have a much higher sulfur content than the coarse particles. It is evident from the results of the table that the use of minus 8-mesh dolomite, including the fine dust, results in a surface coating (small particles have higher sulfur content than large particles) whereas the use of sized dolomite from which the minus 100-mesh particles have been removed does not result in the formation of a surface layer with an appreciable sulfur content on the sponge iron at 1950° F. and is therefore an effective desulfurizing agent.

From a comparison of the data in parts (b) and (c) of the example, it appears that the elimination of the minus 100-mesh fraction of the dolomite prevents the formation of a surface coating and results in a low-sulfur sponge iron.

As shown in the foregoing descriptions and example, iron of a very low sulfur content can be produced by heating iron ore and a suitable carbonaceous reducing agent with sized dolomite as a desulfurizing agent. It has been found that employing unsized dolomite as the desulfurizing agent in such a process results in a much higher sulfur content in the finished iron product.

While the invention has been particularly described in connection with iron production by the sponge method its utility is not limited thereto, since in other processes the reduction of iron ore occurs in a similar manner. The use of properly sized dolomite as a desulfurizing agent in a blast furnace should result in the production of low sulfur iron in the upper portion of the furnace before carburization and melting occur and therefore the metal would not require desulfurization with slags in the lower section of the furnace as occurs in modern practice. With proper design and operation of blast furnaces, such production of low sulfur iron before melting occurs would aid considerably in the manufacture of low sulfur pig iron.

While the invention has been particularly described in relation to the reduction of iron ores, it is likewise useful in the reduction of other metallic ores by means of coke, where it is desirable to have a low sulfur content in the finished metal.

Since many widely differing embodiments of the invention will occur to one skilled in the art, the invention is not limited to the specific details illustrated and described, and various changes can be made therein without departing from the spirit and scope thereof.

What is claimed is:

55 In a process for the production of sponge iron, the steps which comprise forming a reducible mixture of iron ore and a carbonaceous reducing agent, adding thereto dolomite which has been sized to about minus 20 plus 100 mesh, and reducing said mixture.

RUSSELL C. BUEHL.  
JOHN P. RIOTT.  
EARLE P. SHOUB.

REFERENCES CITED

65 The following references are of record in the file of this patent:

UNITED STATES PATENTS

70 Number Name Date  
1,065,890 Sieurin \_\_\_\_\_ June 24, 1913  
2,380,406 Buehl \_\_\_\_\_ July 31, 1945

OTHER REFERENCES

75 "Production of Low Sulphur Sponge Iron,"  
Metals Technology, October 1946 (TP 2093).